# EUROPEAN PATENT SPECIFICATION

(11) **EP 0 364 596 B1**
(45) Date of publication and mention of the grant of the patent: **06.03.1996**
(21) Application number: 89903215.5
(22) Date of filing: 15.03.1989
(51) Int. Cl.: C25D 5/48, C25D 11/34, C23C 22/07

(54) **METHODS FOR PRODUCING Zn-Ni ALLOY-PLATED STEEL SHEET HAVING EXCELLENT PRESS MOLDABILITY**
VERFAHREN ZUR HERSTELLUNG VON MIT ZINK-NICKEL-LEGIERUNG BESCHICHTETEN FEINBLECHEN MIT AUSGEZEICHNETEN PRESSVERFORMEIGENSCHAFTEN
PROCEDES DE PRODUCTION D'UNE FEUILLE D'ACIER A REVETEMENT EN ALLIAGE DE Zn-Ni PRESENTANT UNE EXCELLENTE APTITUDE AU MOULAGE PAR PRESSAGE

(30) Priority: 16.03.1988 JP 60575/88
(43) Date of publication of application: 25.04.1990
(73) Proprietor: KAWASAKI STEEL CORPORATION, Chuo-Ku, Kobe-City Hyogo 651 (JP)
(72) Inventor: MUKO, Ryoichi, Kawasaki-cho Chiba-shi, Chiba 260 (JP); MOCHIZUKI, Kazuo, Kawasaki-cho Chiba-shi, Chiba 260 (JP); KIMURA, Hajime, Kawasaki-cho Chiba-shi, Chiba 260 (JP); ICHIDA, Toshio, Kawasaki-cho Chiba-shi, Chiba 260 (JP)
(74) Representative: Grünecker, August, Dipl.-Ing.
(86) International application number: JP8900276
(87) International publication number: WO8908730

(56) References cited:
- FR-A- 1 581 111
- JP-A- 6 164 884
- JP-A-61 288 098
- JP-B- 4 515 851
- H.W. DETTNER et al.: "Handbuch der Galvanotechnik", Band III, 1969, pages 86- 88, Carl Hanser Verlag, Munich, DE
- WORLD PATENT INDEX LATEST, accession no. 81-86453D/47; & JP-A-56 130 477
- Encyclopedia of Chemical Technology, Kirk-Othmer, 3rd Edn. Vol.15, pages 304 to 307

## Description

### FIELD OF THE INVENTION

This invention relates to methods for producing a Zn-Ni alloy plated steel plate having superior press formability.

### BACKGROUND OF ART

The Zn-Ni alloy plated steel sheet, strip or plate exhibits corrosion resistance about five to ten times that of the Zn-plated steel plate having the same deposited amount of the plated metal. For this reason, it is used in an increasing amount as a steel plate for coping with the problem recently presented of early corrosion of vehicle bodies caused by road freezing preventive agents employed in winter, and is used at various portions from the front fender to a bonnet and trunk lid outer. Also the present-day trend is to use a double side plated steel plate on the outer surface of the vehicle body with the aim of improving the corrosion resistance after peel-off of the coating by the stones or pebbles striking on the outer surface, to replace the one side plated steel plate during the time of early usage of the plated steel plates which was aimed at preventing rusting at the portions where coating may be insufficient, such as the inner surface of the vehicle body.

For preparing the Zn-Ni plated steel plate, there are required properties different from those required of the one side plated plate. Among these properties is the press formability.

In view of the above described usage of the single side plated steel plate, it is a frequent occurrence that the inner side of the punch, that is, the cold rolled surface thereof, turns out to be the protruding surface at the time of press working, so that the plated surface has little effect on the press formability.

However, in the case of the double side plated steel plate, the plated surface turns out to be the protruding surface at the time of press working, and the friction of the plated surface itself presents problems. Although the press working may naturally be facilitated with the use of the highly viscous press oil at the time of press working, the customary practice is to apply the rust preventive oil of low viscosity to the plated steel plate and to perform the press working with the rust preventive oil resting on the plate surface to facilitate the degreasing and coating at the user. The plated plate is required to have satisfactory workability with the rust preventive oil applied thereto.

As the method for improving the press formability of the Zn-Ni alloy plated place, there is known a method consisting in applying a Zn-Ni alloy plating in double layers to increase the Ni contents of the upper layer, as disclosed in the Japanese Patent Application KOKAI No.141394/1985.

This method utilizes the so-called powdering of the upper Zn-Ni plating layer to improve the press workability, the peeled-off powders are placed and heaped on the press mold surface, in case of continuous stamping of a large number of samples, thus causing the problem of pimples.

From JP-A-61-288098 a method is known comprising plating a steel sheet with a Zn-Ni layer and subjecting the plated surface to an anodic treatment in order to blacken said surface. The charge values in said anodic treatment are 100 to 300 C/dm.

From Encyclopedia of Chemistry Technology, Kirk-Othmer, 3rd Edition, vol. 15, pages 304 to 307, it is known to deposit about 2.2 to 11 g/m of phosphate, wherein a zinc-based bath is employed, containing zinc oxide and phosphoric acid to deposit a zinc phosphate coating.

### DISCLOSURE OF THE INVENTION

The present invention contemplates to eliminate the lowering of the press formability caused by the frictional resistance of the plated surface of the Zn-Ni alloy plated steel plate, and is aimed to improve the press formability without accompanying powdering of the plated layer, such as is encountered in the prior art.

Thus, according to the first aspect of the present invention, there is provided a method for producing a Zn-Ni alloy plated steel plate having superior press formability comprising the steps as defined in claim 1.

According to the second aspect of the present invention, there is provided a method for producing a Zn-Ni alloy plated steel plate having superior press formability comprising the steps as defined in claim 2.

According to the third aspect of the present invention, there is provided a method for producing a Zn-Ni alloy plated steel plate having superior press formability comprising the steps as defined in claim 3

### BRIEF DESCRIPTION OF THE DRAWINGS

Fig.1 is a chart showing the limiting drawing ratio (LDR) for illustrating the effect of the present invention following the dipping treatment.

Fig.2 is a chart showing changes of the limiting drawing ratio (LDR) after the dipping treatment.

Fig.3 is a chart showing the result of comparison between the LDR of the Zn-Ni alloy plated plate and that of the cold rolled plate.

Fig.4 is a diagrammatic view showing a cylindrical deep drawing tester.

Fig.5 is a diagrammatic view showing a friction measurement tester.

Fig.6 shows the difference in the friction between the Zn-Ni alloy plated plate and the cold rolled plate.

### BEST EMBODIMENT OF PRACTICING THE INVENTION

The process under which the present invention has been arrived at is first explained.

Fig.3 shows the relative ease with which the cold rolled plate, the single-side Zn-Ni alloy plated steel plate and the double-side Zn-Ni alloy plated steel plate are expressed in terms of the limiting drawing ratio (LDR) in a cylindrical deep drawing testing. The limiting drawing ratio was measured by taking the ratio of the punch diameter to the blank diameter when a test plate is broken as the blank diameter is changed between the values of 60 and 80 mm using a cylindrical deep drawing tester shown in Fig.4. The testing was performed so that the cold rolled surface of the single-side Zn-Ni alloy plated steel plate turned out to be the protruding surface. The rust preventive oil manufactured by the Idemitsu Kosan Co. Ltd. under the registered trade mark of "Daphney Oil Coat" and a predetermined steel plate type corresponding to SPCC was employed to check only for the effects on the plated layer. The amount of deposition on one side of the plated layer was 30 g/m, while the Ni contents were 12.5%.

It is seen from this figure that the double-side plated plate is low in LDR and markedly inferior in press formability as compared with the cold rolled plate. Since the plated steel plate is a substitute material for cold rolled plate, it is pressed on a press mold designed for use with cold rolled plates. It was found that the tested plate was broken on a press mold designed for use exclusively with ultra deep drawing steel plate.

Since it was felt that the low value of LDR of the plated plate could possibly be attributed to the friction on the surface of the plated plate, the frictional resistance on the surface of the plated plate was tentatively measured by a friction measurement tester. The tester used in this test is shown diagrammatically in Fig.5. With this tester, the value of the frictional force is assessed from the value of the load required when a sample in the sandwiched state is tracted at a predetermined traction speed. The testing was performed without lubricant. Fig.6 shows the test results.

It is thought that, as may be seen from this figure, the cold rolled plate differs from the plated plate in surface friction, and this difference possibly affects the formability.

Our eager researches were then directed to clarification of the factors governing the friction coefficient of the plated surface of the Zn-Ni alloy plated steel plate. These researches led to the following finding: i) Changes in the outermost layer of the plated layer result in changes in press formability. ii) The cold rolled plate is not affected markedly in quality as a result of plating.

Our researches were continued with reference to the above feature i) and it was now found that the press formability could be improved markedly by dipping the Zn-Ni plated surface with the use of a solution containing one or both of H₂PO₄ ⁻ ions and HPO₄ ²⁻ ions.

Fig.1 shows the changes in LDR when the Zn-Ni alloy plated plate was dipped for four seconds in the following solution. The amount of deposition on one side of the plated plate was 30 g/m, the Ni contents were 12.5 % and the type of the steel used was SPCC.

| | | |
|---|---|---|
| processing solution | NaH₂PO₄ | 200 g/l |
| | K₂HPO₄ | 150 g/l |
| | temperature | 60°C |
| | pH | 5.8 |

It is seen that treatment by this solution of the plated plate results in improved LDR. The results of glow discharge spectroscopy (GDS) revealed that the P peak exists on the surface of the plated plate following the dipping and that this P on the plated plate surface possibly results in improved lubricating properties and improved press formability.

Based on the above theoretical considerations, the practical construction of the present invention will be explained in more detail.

The solution employed in the dipping treatment may contain one or both of H₂PO₄ ⁻ ions and HPO₄ ²⁻ ions.

Although there is no limitation to the concentration or temperature of the solution, since some time may be involved due to the dipping treatment until the effect is displayed, it is preferred that the temperature and the concentration be elevated for more prompt effects. For short time treatment of less than 10 seconds, suited for industrial production, it is preferred that the dipping temperature be not lower than 40 °C and the concentration in the dipping solution of the H₂PO₄ ⁻ and HPO₄ ²⁻ summed together be not less than 100 g/l.

The Ni contents in the plated plate employed are 10 to 17 wt.% and preferably 11 to 15 wt.%. The contents lower than 10 wt.% are not effective in the case of the present method, while the contents in excess of 17 wt.% tend to cause powdering in the Zn-Ni plated layer. It is for this reason that the Ni contents of the Zn-Ni alloy plated steel plate of the present invention are limited to the range of 10 to 17 wt.%. In the meantime, addition of Co, Fe, Cr, Cu, Mn, Al etc. in an amount of not more than several percent for further improving the corrosion resistance may be made without departing from the purport of the present invention.

The pH of the solution is 4 to 10. With the pH lower than 4, Zn, above all, of the plated layer is dissolved severely thus decreasing the amount of deposition of the plated material. On the other hand, with the pH above 10, the effect in improving the press formability is annulled. It is for this reason that the pH of the solution is limited to 4 to 10.

The positive ions of K⁺, Na⁺, Mg⁺, Ca⁺ or Al³⁺ etc. in the employed solution should be electro-chemically less noble than Zn and Ni. It is because metals electro-chemically less noble than Zn and Ni undergo a substitution reaction with Zn or Ni to be precipitated on the plated surface to degrade the appearance when the plated plate is dipped in a solution containing metal ions. The amount of P on the plated surface, when reckoned as P, is 0.1 to 5 mg/m. With the amount lower than 0.1 mg/m, the effect is annulled. On the other hand, with the amount in excess of 5 mg/m, phosphatability is deteriorated.

The treatment by the solution containing HPO₄ ²⁻ and/or H₂PO₄ ⁻ may also be made by spraying by the above solution, in place of the above described dipping. The operating conditions at this time may be approximately the same as those obtained in the dipping treatment.

Also, for improving the press formability of the Zn-Ni alloy plated steel plate, anodic treatment in the above solution may also be performed in place of the dipping and spraying methods. The conditions for anodic treatment include electric charges of up to 100 c(coulomb)/dm since the plated layer, above all Zn tends to be dissolved in excess of 100 c/dm.

### EXAMPLES

In Table 1, the steel plate samples, plating and dipping conditions and the press formability expressed as LDR, are shown collectively. As the lube oil, the "Daphney Oil Coat Z5" a rust preventive oil manufactured by the Idemitsu Kosan Co. Ltd., was used in all cases.

For Example 1 and Comparative Examples 1 and 2, the LDR values are shown in Fig.2 for more clear demonstration of the effects of the present invention.

The examples of spraying and anodic treatment are also shown in Table 2. It may be seen that the Zn-Ni alloy plated steel plate having stable press formability may be obtained by these treatments as by the above described dipping treatment.

### INDUSTRIAL UTILIZABILITY

According to the present invention, the plated surface of a Zn-Ni alloy plated steel plate is treated by dipping, spraying or by anodic treatment by a solution containing HPO₄ ²⁻ and/or H₂PO₄ ⁻, whereby
i) press formability of the Zn-Ni alloy plated steel plate is improved to the level of the cold rolled plate, and press cracking at the time of press working is eliminated; and
ii) press formability is similar for any contents of Ni within the range of the Ni contents of 10 to 17 wt.%, so that fluctuations in press workability caused by fluctuations in the composition of the plating bath or line speed is eliminated;

so that the Zn-Ni alloy plated steel plate having stable formability may be produced with significant industrial advantages.

## Claims

1. A method for producing a Zn-Ni alloy plated steel plate having superior press formability comprising the steps of plating the surface of a steel plate with a Zn-Ni alloy having the Ni content cf 10 to 17% by weight and subjecting the plated surface to a dipping treatment using a solution at a pH of 4 to 10 containing one or both of H₂PO₄ ⁻ and HPO₄ ²⁻ ions to deposit 0.1 to 5 mg/m cf phosphate calculated as P.

2. A method for producing a Zn-Ni alloy plated steel plate having superior press formability comprising the steps of plating the surface of a steel plate with a Zn-Ni alloy having the Ni contents of 10 to 17% by weight and subjecting the plated surface to a spraying treatment using a solution at a pH of 4 to 10 containing one or both of H₂PO₄ ⁻ and HPO₄ ²⁻ ions to deposit 0.1 to 5 mg/m of phosphate calculated as P.

3. A method for producing a Zn-Ni alloy plated steel plate having superior press formability comprising the steps of plating the surface of a steel plate with a Zn-Ni alloy having the Ni contents of 10 to 17% by weight and subjecting the plated surface to an anodic treatment of up to 100 C/dm using a solution at a pH of 4 to 10 containing one or both of H₂PO₄ ⁻ and HPO₄ ²⁻ ions to deposit 0.1 to 5 mg/m of phosphate calculated as P.

## Patentansprüche

1. Verfahren zur Herstellung von mit Zink-Nickel-Legierung beschichteten Feinblechen mit ausgezeichneten Preßformeigenschaften, bei dem die Oberfläche eines Feinblechs mit einer Zink-Nickel-Legierung mit einem Nickelgehalt von 10 bis 17 Gew.-% beschichtet wird und bei dem die beschichtete Oberfläche einer Tauchbehandlung unter Verwendung einer Lösung mit einem pH-Wert von 4 bis 10, in der H₂PO₄ ⁻- und/oder HPO₄ ²⁻-Ionen enthalten sind, unterzogen wird, um 0,1 bis 5 mg/m Phosphate, bezogen auf P, aufzutragen.

2. Verfahren zur Herstellung von mit Zink-Nickel-Legierung beschichteten Feinblechen mit ausgezeichneten Preßformeigenschaften, bei dem die Oberfläche eines Feinblechs mit einer Zink-Nickel-Legierung mit einem Nickelgehalt von 10 bis 17 Gew.-% beschichtet wird und bei dem die beschichtete Oberfläche einer Spühbehandlung unter Verwendung einer Lösung mit einem pH-Wert von 4 bis 10, in der H₂PO₄ ⁻- und/oder HPO₄ ²⁻-Ionen enthalten sind, unterzogen wird, um 0,1 bis 5 mg/m Phosphate, bezogen auf P, aufzutragen.

3. Verfahren zur Herstellung von mit Zink-Nickel-Legierung beschichteten Feinblechen mit ausgezeichneten Preßformeigenschaften, bei dem die Oberfläche eines Feinblechs mit einer Zink-Nickel-Legierung mit einem Nickelgehalt von 10 bis 17 Gew.-% beschichtet wird und bei dem die beschichtete Oberfläche einer anodischen Behandlung bei bis zu 100 C/dm unter Verwendung einer Lösung mit einem pH-Wert von 4 bis 10, in der H₂PO₄ ⁻-und/oder HPO₄ ²⁻-Ionen enthalten sind, unterzogen wird, um 0,1 bis 5 mg/m Phosphate, bezogen auf P, aufzutragen.

## Revendications

1. Procédé de production d'une tôle d'acier revêtue d'un alliage de Zn-Ni ayant une aptitude supérieure au moulage à pression comprenant les étapes consistant à revêtir la surface d'une tôle d'acier avec un alliage de Zn-Ni ayant une teneur en Ni de 10 à 17% en poids et à soumettre la surface métallisée à un traitement par immersion dans une solution d'un pH de 4 à 10, contenant des ions H₂PO₄- ou HPO₄ ²⁻, ou les deux, de manière à déposer de 0,1 à 5 mg/m de phosphate, calculé en poids de P.

2. Procédé de production d'une tôle d'acier revêtue d'un alliage de Zn-Ni ayant une aptitude supérieure au moulage à pression comprenant les étapes consistant à revêtir la surface d'une tôle d'acier avec un alliage de Zn-Ni ayant une teneur en Ni de 10 à 17% en poids et à soumettre la surface métallisée à un traitement par pulvérisation avec une solution d'un pH de 4 à 10 contenant des ions H₂PO₄- ou HPO₄ ²⁻, ou les deux, de manière à déposer de 0,1 à 5 mg/m2 de phosphate, calculé en poids de P.

3. Procédé de production d'une tôle d'acier revêtue d'un alliage de Zn-Ni ayant une aptitude supérieure au moulage à pression comprenant les étapes consistant à revêtir la surface d'une tôle d'acier avec un alliage de Zn-Ni ayant une teneur en Ni de 10 à 17% en poids et à soumettre la surface métallisée à un traitement anodique allant jusqu'à 100 C/dm dans une solution d'un pH de 4 à 10 contenant des ions H₂PO₄- ou HPO₄ ²⁻, ou les deux, de manière à déposer de 0,1 à 5 mg/m de phosphate, calculé en poids de P.
